# EUROPEAN PATENT SPECIFICATION

(11) **EP 1 761 344 B1**
(45) Date of publication and mention of the grant of the patent: **17.12.2008**
(21) Application number: 05729727.7
(22) Date of filing: 31.03.2005
(51) Int. Cl.: B08B 17/04

(54) **CARGO TANK COATING**
BESCHICHTUNG FÜR LADETANKS
REVETEMENT DE CITERNE DE CHARGE

(30) Priority: 28.06.2004 GB 0414404
(43) Date of publication of application: 14.03.2007
(73) Proprietor: L & I Maritime Ltd, Worksop Nottingham S80 2DE (GB)
(72) Inventor: JOHNSON, Guy, c/o L & I Maritime Ltd., Workshop, Nottingham S80 2DE (GB)
(74) Representative: Franks & Co Limited
(86) International application number: PCT/GB2005/001304
(87) International publication number: WO 2006/000736

(56) References cited:
- EP-A- 0 366 268
- DE-A1- 4 014 909
- GB-A- 404 874
- GB-A- 504 500
- GB-A- 2 237 790

## Description

### Field of the Invention

The present invention relates to a barrier coating formulation coated onto the interior surface of a cargo tank and in particular, although not exclusively, to a water soluble barrier coating configured to form a preventive coating on the interior surface of the cargo tank.

### Background to the Invention

Cargo tankers are used to transport a variety of different cargoes by sea. Commonly, the cargo is in liquid form being stored within large cargo tanks located within the vessel body.

It is possible to divide these cargo tanks into three separate categories based on the type of coating formed on the interior surface of the tank or the type of material from which the tank is manufactured. A known and first type of tank is manufactured from stainless steel, a second type is coated with an organic based coating (e.g. a phenolic based epoxy or polyurethane epoxy) and a third type is coated with an inorganic based coating which is commonly zinc silicate.

EP 0 366 268 discloses a coating for internal surfaces of tanks such as cargo tanks for liquids. These internal surfaces are coated by application of a metal plating compositions such as an electroless plating composition or an electroplating composition to prevent corrosion of the steel tank.

GB 404 874 discloses a protective coating composition for the treatment of interior surfaces of oil containers, such as the oil tanks of ships, comprising a barium sulphate composition to provide a coating which can easily be removed when no longer required and is more stable when stored for a long period of time. Such a coating may be removed from the interior surfaces by steaming.

Cargo vessels are typically required to transport a variety of different liquid cargoes ranging from specialist chemicals to crude hydrocarbon based oils. It is therefore required to thorough clean the interior of the cargo tanks between transportations of different cargos to ensure the liquid cargo is not contaminated by residual amounts of the previous cargo.

Detergents and solvents, in particular, methanol, ethanol and ketones are commonly used to thoroughly clean the interior surfaces. As will be appreciated, a certain amount of cargo penetrates the interior surface of the cargo tank during storage particularly in the case of the organic and inorganic coatings. The problem of cargo penetration and adsorption at the tank surface necessitates extensive cleaning of the internal surface with aggressive detergents and solvents, particularly where the storage and transportion of hydrocarbon oils is concerned.

Moreover, the interior surfaces of zinc silicate coated cargo tanks are typically profiled, whereby hydrocarbons are captured and trapped within micro cavities formed within the coating. These trapped hydrocarbons are not readily removed with detergents and solvents. There are many problems associated with the use of detergents and solvents for the large scale cleaning of cargo tanks including for example hazardous working conditions for personnel cleaning the tanks, and storage and disposal of the cleaning products before and after use.

A further problem exists with conventional cleaning techniques due to the incomplete removal of cargo from the interior surfaces particularly where hydrocarbon based cargoes have been transported. Incomplete cargo removal results in both subsequent cargo contamination and significant delays in transportation resulting from extended cleaning operations. What is required therefore is apparatus and method to solve the above problems.

### Summary of the Invention

A barrier coating formulation is provided configured as a preventive coating for the interior surface of a cargo tank whereby hydrocarbon based cargoes are prevented from adhering to the interior surface during and after transportation. The interior surfaces of the cargo tanks, coated with the formulation according to the present invention, require considerably less time intensive cleaning operations when compared to untreated tanks. Moreover, the requirement for strong detergents and aggressive solvents, as part of the cleaning operation is avoided.

The preventive coating is water soluble and may be removed from the interior surface by rinsing with water, in particular hot water. Moreover, the formulation according to a specific implementation of the present invention comprises. naturally occurring compounds and therefore provides numerous environmental advantages.

According to a first aspect of the present invention there is provided a cargo tank of a sea going vessel, said cargo tank having a primary coating on its interior surface and a secondary temporary coating coated onto said primary coating, said secondary coating comprising: a solvent; and a rheological additive configured to increase the viscosity of said solvent; wherein said secondary coating comprises a viscosity configured to provide temporary adhesion to said primary coating, said secondary coating serving as a temporary barrier coating to prevent a liquid cargo transported within said cargo tank from absorbing at said primary coating, said secondary coating capable of being removed from said cargo tank after transportation of said cargo by rinsing said interior surface with water.

According to a second aspect of the present invention there is provided a use of a formulation comprising a solvent and a rheological additive configured to increase the viscosity of said solvent as a secondary temporary barrier coating coated onto a primary coating provided on an interior surface on a cargo tank of a sea going vessel; wherein said secondary coating comprises a viscosity configured to provide temporary adhesion to said primary coating, said secondary coating serving as a temporary barrier coating to prevent liquid cargo transported within said cargo tank from adsorbing at said primary coating, said secondary coating capable of being removed from said cargo tank after transportation of said cargo by rinsing said interior surface with water.

According to a third aspect of the present invention there is provided a method of preventing hydrocarbon based liquid cargo from adsorbing at a primary coating coated onto an interior surface of a cargo tank of a sea going vessel, said method comprising: mixing a solvent comprising at least one hydroxyl group with a rheological additive configured to increase the viscosity of said solvent to form a water soluble barrier coating formulation: coating said primary coating of said cargo tank with said water soluble barrier coating formulation to form a secondary temporary coating; storing a hydrocarbon based liquid cargo within said cargo tank; removing said hydrocarbon based liquid from said tank; and removing said secondary coating from said interior surface by washing said interior surface with water; wherein said secondary coating comprises a viscosity configured to provide temporary adhesion to said primary coating, said secondary coating serving as a temporary barrier coating to prevent said liquid cargo from adsorbing to said primary coating.

### Detailed Description

There will now be described by way of example a specific mode contemplated by the inventors. In the following description numerous specific details are set forth in order to provide a thorough understanding. It will be apparent however, to one skilled in the art, that the present invention may be practiced without limitation to these specific details. In other instances, well known methods and structures have not been described in detail so as not to unnecessarily obscure the description.

The inventors provide a water soluble barrier coating formulation and a method of coating an interior surface of a cargo tank with a formulation so as to considerably inhibit a hydrocarbon or hydrocarbon based cargo penetrating and adhering to the interior surface of a cargo tank.

The preventative coating comprising the rheological additive, is sufficiently viscous whereby during application of the formulation in the liquid phase it is configured to adhere to the cargo tank surface and not drain away under gravity. Once applied, the formulation is configured to dry forming a substantially solid barrier coating.

The formulation is particularly advantageous for coating zinc silicate cargo tank surfaces in that micro cavities or pores formed within the zinc silicate may be filled or blocked by the formulation during application in the liquid phase and subsequent drying to form a solid coating. The zinc silicate coating is thereby not exposed to the cargo during storage and transportation.

As the water soluble formulation is substantially insoluble in hydrocarbon oils the formulation is particularly advantageous as a barrier coating for the transportation of hydrocarbons and hydrocarbon based oils.

### Formulations

The following examples include different alternative barrier coating formulations configured to be particularly suitable as prevented coatings for the interior surfaces of cargo tanks. In particular, the examples detailed herein may be utilised with a variety of different cargo tank types including, for example, stainless steel cargo tanks, zinc silicate coated cargo tanks and cargo tanks initially coated with organic and/or inorganic paints.

Accordingly, the present invention is not restricted to anyone of the following examples and in particular may include combinations of different examples.

### Example 1

A barrier coating formulation comprising water and one or more natural gum selected from the list of:
- carrageenan gum;
- xanthan gum;
- arabic gum;
- tragacanth gum;
- guar gum;
- caroube gum;
- pectin

### Example 2

A water soluble barrier coating formulation comprising water and one or a combination of cellulosics selected from the list of:
- carboxmethyl cellulose (CMC);
- hydroxyethyl cellulose (HEC);
- hydrophobically modified (HEC);
- methyl cellulose (MC);
- methyl hydroxyethyl cellulose (MHEC);
- methyl hydroxpropyl cellulose (MHPC);
- ethyl hydroxyethyl cellulose (EHEC);
- hydrophobically modified (EHEC) or (HM-EHEC).

### Example 3

A water soluble barrier coating formulation comprising water and anyone or a combination of organoclays selected from the list of:
- bentonite;
- hectorite

### Example 4

A water soluble barrier coating formulation comprising water and a gellant, in particular gelatine.

### Example 5

A water soluble barrier coating formulation comprising water and one or a combination of associative synthetics selected from the list of:
- an aqueous swellable emulsion (HASIE);
- a polyurethane based thickener (HEUR);
- a hydrophobically modified polyether.

### Example 6

A water soluble barrier coating formulation comprising water and polyviriylalcohol.

### Example 7

A water soluble barrier coating formulation comprising water and starch or a starch derivative.

### Example 8

A water soluble barrier coating formulation comprising glycerol or a glycerol derivative and one or more natural gum selected from the list of:
- carrageenan gum;
- xanthan gum;
- arabic gum;
- tragacanth gum;
- guar gum;
- caroube gum;
- pectin.

### Example 9

A water soluble barrier coating formulation comprising glycerol or a glycerol derivative, in particular monoethylene glycol, and one or a combination of cellulosics selected from the list of:
- carboxmethyl cellulose (CMC);
- hydroxyethyl cellulose (HEC);
- hydrophobically modified (HEC);
- methyl cellulose (MC);
- methyl hydroxyethyl cellulose (MHEC);
- methyl hydroxpropyl cellulose (MHPC);
- ethyl hydroxyethyl cellulose (EHEC);
- hydrophobically modified (EHEC) or (HM-ENEC).

### Example 10

A water soluble barrier coating formulation comprising glycerol or a glycerol derivative, and anyone or a combination of organoclays selected from the list of:
- bentonite;
- hectorite.

### Example 11

A water soluble barrier coating formulation comprising glycerol or a glycerol derivative, and a gellant, in particular gelatin.

### Example 12

A water soluble barrier coating formulation comprising glycerol or a glycerol derivative, and one or a combination of associative synthetics selected from the list of:
- an aqueous swellable emulsion (HASIE);
- a polyurethane based thickener (HEUR);
- a hydrophobically modified polyether.

### Example 13

A water soluble barrier coating formulation comprising glycerol or a glycerol derivative, and polyvinylalcohol.

### Example 14

A water soluble barrier coating formulation comprising glycerol or a glycerol derivative and starch or a starch derivative.

### Example 15

A water soluble barrier coating formulation comprising glycerol or a glycerol derivative, pectin and xanthan gum.

### Example 16

A water soluble barrier coating formulation comprising glycerol or a glycerol derivative, polyvinylalcohol and xanthan gum.

### Example 17

A water soluble barrier coating formulation comprising glycerol or a glycerol derivative, carrageenan gum and xanthan gum.

### Example 18

A water soluble barrier coating formulation comprising glycerol or a glycerol derivative, gelatin and xanthan gum.

### Cargo Tank Coating

### Example 1

The water, glycerol or glycerol derivative solvent is firstly mixed with the rheological additive in sufficient proportions whereby the viscosity of the resulting mixture is sufficient to provide temporary adhesion of the formulation to the interior surface of the cargo tank during a drying process such that the liquid formulation is inhibited from draining away under gravity. The interior surface of the cargo tank may comprise stainless steel, an organic based paint or an inorganic coating being, in particular, zinc silicate. The formulation is then sprayed onto the interior surface using a mechanical spray device being a motorised spray apparatus for example a fuel or pneumatically driven device.

The viscosity of the substantially liquid formulation comprises a viscosity suitable to enable the formulation to be sprayed onto the interior surface of the cargo tank. In particular, the viscosity may be tailored by variation of the chosen rheological additive, the amount of rheological additive and/or the combinations of rheological additives included within the formulation. Moreover, the temperature of the formulation may be selectively adjusted during application onto the interior surface of the tank in order to optimise coverage of the surface whilst ensuring the formulation does not drain away under gravity once applied.

According to the specific implementations of the present invention the viscosity of the liquid phase formulation may be either proportional or inversely proportional to temperature.

Depending upon the type of cargo tank surface to be coated, the pH of the formulation may be tailored by variation of the rheological additive, with regard to compound, quantity, combinations thereof and/or temperature, in order to optimise the physical properties of the coating to successfully inhibit contact and penetration of the cargo into the cargo tank surface. In particular, the formulation may comprise a pH within the range 5 to 9 and/or or may be selectively adjusted by the addition of further reagents to sit within this range. Additionally, the formulation may be configured with a pH of 3.

After the internal surface is coated with the formulation, cargo is introduced into the cargo tank wherein it is temporarily stored during transportation. Following transportation, the cargo is removed from the cargo tank. To remove residual cargo from the interior surface in addition to removal of the preventative water soluble barrier coating formulation, the interior surface is washed with water, in particular hot water. The interior surface is then dried before a replacement barrier coating formulation is introduced onto the interior surface in preparation for transportation of a subsequent cargo.

### Example 2

According to a further specific implementation of coating the interior surface of the cargo tank with the barrier coating formulation as illustrated under example 1 immediately above, the formulation may be sprayed onto the interior surfaces by a manual spraying action, for example through the use of a lance spray.

### Example 3

According to a further specific implementation of coating the interior surface of the cargo tank, application of the coating may also be implemented using a fixed or portable tank cleaning machine commonly house within the cargo vessel. The formulation may be applied to the tank surface using the tank cleaning machines via a means of injection or recirculation of the formulation through the vessel's deepwell pump system. As will be appreciated by those skilled in the art, the deepwell pump is configured to pump and remove liquid from the cargo tanks.

According to further specific implementations the barrier coating formulation may be applied to the interior surface using any manor of coating application methods involving the use of brushes, rollers, pads, piping or hoses.

## Claims

1. A cargo tank of a sea going vessel, said cargo tank having a primary coating on its interior surface and a secondary temporary coating coated onto said primary coating, said secondary coating comprising:
a solvent; and
a rheological additive configured to increase the viscosity of said solvent;
wherein said secondary coating comprises a viscosity configured to provide temporary adhesion to said primary coating, said secondary coating serving as a temporary barrier coating to prevent a liquid cargo transported within said cargo tank from adsorbing at said primary coating, said secondary coating capable of being removed from said cargo tank after transportation of said cargo by rinsing said interior surface with water.

2. The cargo tank as claimed in claim 1 wherein said rheological additive is a natural gum comprising any one or a combination of the following set of:
• carrageenan gum;
• xanthan gum;
• arabic gum;
• tragacanth gum;
• guar gum;
• caroube gum;
• pectin.

3. The cargo tank as claimed in claim 1 wherein said rheological additive is cellulose or a cellulose derivative comprising any one or a combination of the following set of:
• carboxymethyl cellulose (CMC);
• hydroxyethyl cellulose (HEC);
• hydrophobically modified (HEC);
• methyl cellulose (MC);
• methyl hydroxyethyl cellulose (MHEC);
• methyl hydroxypropyl cellulose (MHPC);
• ethyl hydroxyethyl cellulose (EHEC);
• hydrophobically modified (EHEC) or (HM-EHEC).

4. The cargo tank as claimed in claim 1 wherein said rheological additive is selected from the group comprising gellants, in particular gelatine, starch derivates, and polyvinylalcohols.

5. The cargo tank as claimed in claim 1 wherein said rheological additive is an associative synthetic comprising any one or a selection of the following set of:
• an aqueous swellable emulsion (HASE);
• a polyurethane based thickener (HEUR);
• a hydrophobically modified polyether.

6. The cargo tank as claimed in any preceding claim wherein said solvent selected from the group comprising: water, glycerols and glycerol derivatives, in particular monoethylene glycol.

7. A use of a formulation comprising a solvent and a rheological additive configured to increase the viscosity of said solvent as a secondary temporary barrier coating coated onto a primary coating provided on an interior surface of a cargo tank of a sea going vessel;
wherein said secondary coating comprises a viscosity configured to provide temporary adhesion to said primary coating, said secondary coating serving as a temporary barrier coating to prevent liquid cargo transported within said cargo tank from adsorbing at said primary coating, said secondary coating capable of being removed from said cargo tank after transportation of said cargo by rinsing said interior surface with water.

8. The use of said formulation as claimed in claim 6 wherein said solvent is selected from the group comprising water, glycerols or glycerol derivatives.

9. A method of preventing a hydrocarbon based liquid cargo from adsorbing at a primary coating coated onto an interior surface of a cargo tank of a sea going vessel, said method comprising:
mixing a solvent comprising at least one hydroxyl group with a rheological additive configured to increase the viscosity of said solvent to form a water soluble barrier coating formulation;
coating said primary coating of said cargo tank with said water soluble barrier coating formulation to form a secondary temporary coating;
storing said hydrocarbon based liquid cargo within said cargo tank;
removing said hydrocarbon based liquid from said tank; and
removing said secondary coating from said interior surface by washing said interior surface with water;
wherein said secondary coating comprises a viscosity configured to provide temporary adhesion to said primary coating, said secondary coating serving as a temporary barrier coating to prevent said liquid cargo from adsorbing to said primary coating.

10. The method as claimed in claim 9 wherein said step of coating said primary coating with said formulation comprises spraying said formulation onto said primary coating.

11. The method as claimed in any one of claims 9 to 10 wherein said solvent selected from the group comprising water, glycerols or glycerol derivatives.

12. The method as claimed in claim 11 wherein said rheological additive is a natural gum comprising any one or a combination of the following set of:
• carrageenan gum;
• xanthan gum;
• arabic gum;
• tragacanth gum;
• guar gum;
• caroube gum;
• pectin.

13. The method as claimed in claim 11 wherein said rheological additive is cellulose or a cellulose derivative comprising any one or a combination of the following set of:
• carboxymethyl cellulose (CMC);
• hydroxyethyl cellulose (HEC);
• hydrophobically modified (HEC);
• methyl cellulose (MC);
• methyl hydroxyethyl cellulose (MHEC);
• methyl hydroxypropyl cellulose (MHPC);
• ethyl hydroxyethyl cellulose (EHEC);
• hydrophobically modified (EHEC) or (HM-EHEC).

14. The method as claimed in claim 11 wherein said rheological additive is an associative synthetic comprising any one or a selection of the following set of:
• an aqueous swellable emulsion (HASE);
• a polyurethane based thickener (HEUR);
• a hydrophobically modified polyether.

15. The method as claimed in claim 11 wherein said rheological additive is selected from the group comprising polyvinylalcohols, and gellants, in particular gelatin.

## Patentansprüche

1. Ladetank eines Seeschiffs, wobei der genannte Ladetank eine Primärbeschichtung auf seiner Innenfläche und eine auf die genannte Primärbeschichtung aufgetragene temporäre Sekundärbeschichtung hat, wobei die genannte Sekundärbeschichtung Folgendes umfasst:
ein Lösungsmittel und
einen rheologischen Zusatzstoff, der so konfiguriert ist, dass er die Viskosität des genannten Lösungsmittels erhöht,
wobei die genannte Sekundärbeschichtung eine Viskosität aufweist, die so konfiguriert ist, dass eine temporäre Adhäsion an der genannten Primärbeschichtung erreicht wird, wobei die genannte Sekundärbeschichtung als eine temporäre Sperrbeschichtung dient, um eine in dem genannten Ladetank transportierte flüssige Ladung an einer Adsorption an der genannten Primärbeschichtung zu hindern, wobei die genannte Sekundärbeschichtung nach dem Transport der genannten Ladung durch Abspülen der genannten Innenfläche mit Wasser von dem genannten Ladetank entfernt werden kann.

2. Ladetank nach Anspruch 1, wobei der genannte rheologische Zusatzstoff ein Naturgummi ist, der einen oder eine Kombination der Folgenden umfasst:
• Carrageen-Gummi,
• Xanthangummi,
• Gummiarabikum,
• Tragacanthgummi,
• Guargummi,
• Johannisbrotgummi,
• Pektin.

3. Ladetank nach Anspruch 1, wobei der genannte rheologische Zusatzstoff Cellulose oder ein Cellulosederivat ist, umfassend einen oder eine Kombination der Folgenden:
• Carboxymethylcellulose (CMC),
• Hydroxyethylcellulose (HEC),
• hydrophob modifizierte (HEC),
• Methylcellulose (MC),
• Methylhydroxyethylcllulose (MHEC),
• Methylhydroxypropylcellulose (MHPC),
• Ethylhydroxyethylcellulose (EHEC),
• hydrophob modifizierte (EHEC) oder (HM-EHEC).

4. Ladetank nach Anspruch 1, wobei der genannte rheologische Zusatzstoff ausgewählt ist aus der Gruppe bestehend aus Geliermitteln, insbesondere Gelatine, Stärkederivaten und Polyvinylalkoholen.

5. Ladetank nach Anspruch 1, wobei der genannte rheologische Zusatzstoff ein assoziativer Kunststoff ist, der einen beliebigen oder eine Auswahl der Folgenden umfasst:
• eine wässrige quellfähige Emulsion (HASE),
• einen Verdicker auf Polyurethanbasis (HEUR),
• einen hydrophob modifizierten Polyether.

6. Ladetank nach einem der vorherigen Ansprüche, wobei das genannte Lösungsmittel ausgewählt ist aus der Gruppe bestehend aus Wasser, Glycerolen und Glycerolderivaten, insbesondere Monoethylenglykol.

7. Verwendung einer Formulierung, die ein Lösungsmittel und einen rheologischen Zusatzstoff umfasst, der so konfiguriert ist, dass er die Viskosität des genannten Lösungsmittels erhöht, als eine temporäre Sekundärsperrbeschichtung, die auf eine Primärbeschichtung auf einer Innenfläche eines Ladetanks eines Seeschiffes aufgetragen wird,
wobei die genannte Sekundärbeschichtung eine Viskosität aufweist, die so konfiguriert ist, dass eine temporäre Adhäsion an der genannten Primärbeschichtung erreicht wird, wobei die genannte Sekundärbeschichtung als eine temporäre Sperrbeschichtung dient, um eine in dem genannten Ladetank transportierte flüssige Ladung an einer Adsorption an der genannten Primärbeschichtung zu hindern, wobei die genannte Sekundärbeschichtung nach dem Transport der genannten Ladung durch Abspülen der genannten Innenfläche mit Wasser von dem genannten Ladetank entfernt werden kann.

8. Verwendung der genannten Formulierung nach Anspruch 6, wobei das genannte Lösungsmittel ausgewählt ist aus der Gruppe bestehend aus Wasser, Glycerolen oder Glycerolderivaten.

9. Verfahren zum Verhindern der Adsorption einer flüssigen Ladung auf Kohlenwasserstoffbasis an einer auf einer Innenfläche eines Ladetanks eines Seeschiffes aufgetragenen Primärbeschichtung, wobei das genannte Verfahren die folgenden Schritte beinhaltet:
Mischen eines Lösungsmittels, das wenigstens eine Hydroxylgruppe umfasst, mit einem rheologischen Zusatzstoff, der so konfiguriert ist, dass er die Viskosität des genannten Lösungsmittels erhöht, um eine wasserlösliche Sperrbeschichtungsformulierung zu bilden,
Beschichten der genannten Primärbeschichtung des genannten Ladetanks mit der genannten wasserlöslichen Sperrbeschichtungsformulierung, um eine temporäre Sekundärbeschichtung zu bilden,
Lagern der genannten flüssigen Ladung auf Kohlenwasserstoffbasis in dem genannten Ladetank,
Entfernen der genannten Flüssigkeit auf Kohlenwasserstoffbasis aus dem genannten Tank und
Entfernen der genannten Sekundärbeschichtung von der genannten Innenfläche durch Waschen der genannten Innenfläche mit Wasser,
wobei die genannte Sekundärbeschichtung eine Viskosität aufweist, die so konfiguriert ist, dass eine temporäre Adhäsion an der genannten Primärbeschichtung erreicht wird, wobei die genannte Sekundärbeschichtung als temporäre Sperrbeschichtung dient, um die genannte flüssige Ladung an einer Adsorption an der genannten Primärbeschichtung zu hindern.

10. Verfahren nach Anspruch 9, wobei der genannte Schritt des Beschichtens der genannten Primärbeschichtung mit der genannten Formulierung das Sprühen der genannten Formulierung auf die genannte Primärbeschichtung beinhaltet.

11. Verfahren nach einem der Ansprüche 9 bis 10, wobei das genannte Lösungsmittel ausgewählt wird aus der Gruppe bestehend aus Wasser, Glycerolen oder Glycerolderivaten.

12. Verfahren nach Anspruch 11, wobei der genannte rheologische Zusatzstoff ein Naturgummi ist, der einen oder eine Kombination der Folgenden umfasst:
• Carrageen-Gummi,
• Xanthangummi,
• Gummiarabikum,
• Tragacanthgummi,
• Guargummi,
• Johannisbrotgummi,
• Pektin.

13. Verfahren nach Anspruch 11, wobei der genannte rheologische Zusatzstoff Cellulose oder ein Cellulosederivat ist, umfassend einen oder eine Kombination der Folgenden:
• Carboxymethylcellulose (CMC),
• Hydroxyethylcellulose (HEC),
• hydrophob modifizierte (HEC),
• Methylcellulose (MC),
• Methylhydroxyethylcellulose (MHEC),
• Methylhydroxypropylcellulose (MHPC),
• Ethylhydroxyethylcellulose (EHEC),
• hydrophob modifizierte (EHEC) oder (HM-EHEC).

14. Verfahren nach Anspruch 11, wobei der genannte rheologische Zusatzstoff ein assoziativer Kunststoff ist, der einen oder eine Auswahl der Folgenden umfasst:
• eine wässrige quellfähige Emulsion (HASE),
• einen Verdicker auf Polyurethanbasis (HEUR),
• einen hydrophob modifizierten Polyether.

15. Verfahren nach Anspruch 11, wobei der genannte rheologische Zusatzstoff ausgewählt wird aus der Gruppe bestehend aus Polyvinylalkoholen und Geliermitteln, insbesondere Gelatine.

## Revendications

1. Citerne de charge d'un navire de haute mer, ladite citerne de charge comportant un revêtement primaire sur sa surface interne alors qu'un revêtement secondaire temporaire est appliqué sur ledit revêtement primaire, ledit revêtement secondaire comprenant :
un solvant ; et
un additif rhéologique qui est conçu pour accroître la viscosité dudit solvant ;
cas dans lequel ledit revêtement secondaire possède une viscosité qui est conçue pour procurer une adhérence temporaire audit revêtement primaire, alors que ledit revêtement secondaire joue le rôle de revêtement-barrière temporaire pour éviter qu'une cargaison liquide transportée dans ladite citerne de charge ne soit soumise à un effet d'adsorption au niveau dudit revêtement primaire, ledit revêtement secondaire étant apte à être éliminé de ladite citerne de charge après l'opération de transport de ladite cargaison grâce à un rinçage de ladite surface interne avec de l'eau.

2. Citerne de charge selon la revendication 1, ledit additif rhéologique étant une gomme naturelle constituée de l'une quelconque ou d'une combinaison des substances de l'énumération suivante :
• gomme de carraghénane ;
• gomme de xanthane ;
• gomme arabique ;
• gomme adragante ;
• gomme de guar ;
• gomme de caroube ;
• pectine.

3. Citerne de charge selon la revendication 1, ledit additif rhéologique étant une cellulose ou un dérivé cellulosique constitué de l'une quelconque ou d'une combinaison des substances de l'énumération suivante :
• carboxyméthyl-cellulose (CMC) ;
• hydroxyéthyl-cellulose (HEC) ;
• HEC modifiée hydrophobiquement ;
• méthyl-cellulose (MC) ;
• methyl-hydroxyéthyl-cellulose(MHEC)
• méthyl-hydroxypropyl-cellulose (MHPC) ;
• éthyl-hydroxyéthyl-cellulose (EHEC) ;
• EHEC ou HM-EHEC modifiée hydrophobiquement.

4. Citerne de charge selon la revendication 1, ledit additif rhéologique étant sélectionné parmi le groupe comprenant des gélifiants, en particulier la gélatine, les dérivés de l'amidon et les alcools polyvinyliques.

5. Citerne de charge selon la revendication 1, ledit additif rhéologique étant une matière synthétique associative constituée de l'une quelconque ou d'une sélection des substances de l'énumération suivante :
• une émulsion aqueuse susceptible de gonfler (HASE) ;
• un épaississant à base de polyuréthane (HEUR) ;
• un polyéther modifié hydrophobiquement.

6. Citerne de charge selon l'une quelconque des revendications précédentes, ledit solvant étant sélectionné parmi le groupe constitué des substances suivantes : eau, glycérols et dérivés du glycérol, en particulier le monoéthylène glycol.

7. Utilisation d'une formulation composée d'un solvant et d'un additif rhéologique qui est conçu pour accroître la viscosité dudit solvant sous forme de revêtement-barrière secondaire temporaire qui est appliqué sur un revêtement primaire prévu sur une surface interne d'une citerne de charge d'un navire de haute mer ;
cas dans lequel ledit revêtement secondaire possède une viscosité qui est conçue pour procurer une adhérence temporaire audit revêtement primaire, alors que ledit revêtement secondaire joue le rôle de revêtement-barrière temporaire pour éviter qu'une cargaison liquide transportée dans ladite citerne de charge ne soit soumise à un effet d'adsorption au niveau dudit revêtement primaire, ledit revêtement secondaire étant apte à être éliminé de ladite citerne de charge après l'opération de transport de ladite cargaison grâce à un rinçage de ladite surface interne avec de l'eau.

8. Utilisation de ladite formulation selon la revendication 6, ledit solvant étant sélectionné parmi le groupe constitué des substances suivantes : eau, glycérols ou dérivés du glycérol.

9. Procédé permettant d'empêcher tout effet d'adsorption d'une cargaison liquide, à base d'hydrocarbures, au niveau d'un revêtement primaire appliqué sur une surface interne d'une citerne de charge d'un navire de haute mer, ledit procédé comprenant les étapes consistant à :
mélanger un solvant comprenant au moins un groupe hydroxyle à un additif rhéologique lequel est conçu pour accroître la viscosité dudit solvant afin de constituer une formulation de revêtement-barrière soluble à l'eau ;
enduire ledit revêtement primaire de ladite citerne de charge avec ladite formulation de revêtement-barrière soluble à l'eau afin de constituer un revêtement secondaire temporaire ;
stocker ladite cargaison liquide à base d'hydrocarbures, dans ladite citerne de charge ;
décharger, de ladite citerne, ledit liquide à base d'hydrocarbures ; et
éliminer ledit revêtement secondaire de ladite surface interne grâce à un lavage à l'eau de ladite surface interne ;
cas dans lequel ledit revêtement secondaire possède une viscosité qui est conçue pour procurer une adhérence temporaire audit revêtement primaire, alors que ledit revêtement secondaire joue le rôle de revêtement-barrière temporaire pour éviter que ladite cargaison liquide ne soit soumise à un effet d'adsorption au niveau dudit revêtement primaire.

10. Procédé selon la revendication 9, ladite étape consistant à enduire ledit revêtement primaire avec ladite formulation comprenant l'opération de pulvérisation de ladite formulation sur ledit revêtement primaire.

11. Procédé selon l'une quelconque des revendications 9 à 10, ledit solvant étant sélectionné parmi le groupe constitué des substances suivantes : eau, glycérols ou dérivés du glycérol.

12. Procédé selon la revendication 11, ledit additif rhéologique étant une gomme naturelle constituée de l'une quelconque ou d'une combinaison des substances de l'énumération suivante :
• gomme de carraghénane ;
• gomme de xanthane ;
• gomme arabique ;
• gomme adragante ;
• gomme de guar ;
• gomme de caroube ;
• pectine.

13. Procédé selon la revendication 11, ledit additif rhéologique étant une cellulose ou un dérivé cellulosique constitué de l'une quelconque ou d'une combinaison des substances de l'énumération suivante :
• carboxyméthyl-cellulose (CMC) ;
• hydroxyéthyl-cellulose (HEC) ;
• HEC modifiée hydrophobiquement ;
• méthyl-cellulose (MC) ;
• méthyl-hydroxyéthyl-cellulose (MHEC) ;
• méthyl-hydroxypropyl-cellulose (MHPC) ;
• éthyl-hydroxyéthyl-cellulose (EHEC) ;
• EHEC ou HM-EHEC modifiée hydrophobiquement.

14. Procédé selon la revendication 11, ledit additif rhéologique étant une matière synthétique associative constituée de l'une quelconque ou d'une sélection des substances de l'énumération suivante :
• une émulsion aqueuse susceptible de gonfler (HASE) ;
• un épaississant à base de polyuréthane (HEUR) ;
• un polyéther modifié hydrophobiquement.

15. Procédé selon la revendication 11, ledit additif rhéologique étant sélectionné parmi le groupe comprenant des alcools polyvinyliques et des gélifiants, en particulier la gélatine.
